

Patented July 24, 1928.

1,678,580

# UNITED STATES PATENT OFFICE.

WILHELM WINTERHALDER, OF FRANKFORT-ON-THE-MAIN, GERMANY, ASSIGNOR TO GRASSELLI DYESTUFF CORPORATION, OF NEW YORK, N. Y., A CORPORATION OF DELAWARE.

## PROCESS OF DYEING WITH VAT AND AZO DYESTUFFS.

No Drawing. Application filed May 15, 1926, Serial No. 109,351, and in Germany May 20, 1925.

This invention relates to a process of dyeing cotton, artificial silk and silk with vat- and insoluble azo dyestuffs which process consists in grounding the goods with an azo component and at the same time with a vat dyestuff which has been dissolved by one of the customary methods, and converting the vat dyestuff into the insoluble form by oxidation, and developing the ice color on the fiber by means of a diazo solution.

The azo component deposited on the fiber is rendered more insensitive to the influence of air in a surprising manner by the action of the vat dyestuff. An equi-molecular amount of formaldehyde can nevertheless be added to the padding liquor, and in this case the natural assumption that hydrosulfite adds itself to the formaldehyde whereby the protective action would be taken from the formaldehyde and the vat precipitated at the same time is not proved to be correct.

In this manner uniform dyeings which in case of heavy dyeings are superior in fastness to washing, boiling and rubbing to dyeings made with the vat dyestuff only are obtained with less consumption of dyestuff and a complete exhaustion of the vat dyestuff from the dye bath. In this manner a whole series of shades according to samples can be obtained which can be produced neither with ice colors nor with vat dyestuffs alone. The process is therefore capable of being carried out extremely easily and simply in the usual apparatus.

The process can be used on cotton, artificial silk and surprisingly on natural silk, on degummed silk as well as on silk which has not previously been de-gummed. In the latter case, the silk may be de-gummed during the dyeing process or afterwards. It is surprising that no injury to the silk with respect to luster, strength and touch occurs in spite of attack in a grounding and diazo bath, although the amount of alkali in the grounding bath is considerable and in addition hydrosulfite which is known to be harmful to animal fibers is present.

Vat dyestuffs of all classes may be used for the process of this invention. The process involving the use of vat dyestuffs dissolved by esterification such as the leuco-derivatives described in U. S. Patent 1,448,251 is covered in the application of Petzold and Rittner, Serial No. 39,377. The present

invention relates only to the use of vat dyestuffs dissolved by one of the customary methods and does not include vat dyestuffs dissolved by esterification. As azo components may be used the naphthols, acylamino-naphthols such as benzoylaminonaphthols and the ureas from the 2-5-aminonaphthol-7-sulfonic acid, the derivatives of 1-hydroxynaphthalene-4-carboxylic acid mentioned in U. S. Patent 1,453,660; the arylids of the 2-3-hydroxynaphthoic acid, substances containing a methylene group which is capable of coupling with diazo compounds, also for example pyrazolone derivatives or derivatives of  $\beta$ -ketone-aldehydes, such as the acyl acetic acid arylids, the di- and the mono-acyl acetic acid arylids mentioned in French Patent 567,284, and others.

The invention is illustrated by the following examples:

*Example 1.*—800 gr. of diacetoacetyl-o-tolidine are stirred into a paste with 3 liters of 38° Bé. caustic soda and 1500 gr. of Turkey-red oil, then dissolved in 15 liters of hot water with boiling and diluted to 200 liters. 10 kg. of wetted cotton are introduced at 45° C. and after ten minutes 1.5 kg. of 4,4'-dioxy-indanthrene and 800 gr. of concentrated hydrosulfite powder are added. After a half hour the cotton is hung up for a short time, centrifuged and developed with the following solution:

160 gr. of 2-5-dichloraniline are boiled in 1 liter of water, dissolved with the addition of 310 cc. of 20° Bé. hydrochloric acid, quickly stirred into 1.6 liters of cold water, 1.6 kg. of ice and 310 cc. of 20° Bé. hydrochloric acid. Immediately 80 gr. of sodium nitrite dissolved in 300 cc. of water are added with violent stirring. The mixture is neutralized after 10 minutes with 145 gr. of precipitated chalk and 125 gr. of sodium acetate, dissolved in 700 cc. of water, and then 6 kg. of Glauber's salt and 700 cc. of 50% acetic acid are added. The bath is made up to 200 liters.

After the usual subsequent treatment for vat and azo dyestuffs, a beautiful green is obtained.

*Example 2.*—400 gr. of 2-3-hydroxynaphthoyl-amino-hydroquinone-dimethylether are stirred into a paste with 1000 cc. of 40° Bé. caustic soda and 800 cc. of Turkey-red oil and dissolved with the addition of 40 liters

of water; 133 cc. of 30% formaldehyde solution are added to this solution at 50° C., and then 160 liters of water and 4 liters of sulfite waste liquor are added.

5 The mixture is allowed to stand for a half hour and 10 kg. of cotton are introduced at 30° C. After several minutes there are added 100 gr. of trichlorindanthrene vatted in 10 liters of water, 1 liter of 40° Bé. 10 caustic soda and 500 gr. of concentrated hydrosulfite powder.

The material is thoroughly dyed for half an hour, hung up, squeezed out, centrifuged and developed with the following solution:

15 100 gr. of 2-5-dichloraniline are dissolved in 600 cc. of hot water and 186 cc. of 20° Bé. hydrochloric acid, 1 liter of cold water, 1 kg. of ice, 186 cc. of 20° Bé. hydrochloric acid and 47 gr. of sodium nitrite in 200 cc. 20 of water are added. The mixture is neutralized with 90 gr. of precipitated chalk and 90 gr. of sodium acetate and then 90 gr. of 50% acetic acid and 6 kg. of Glauber's salt are added. The bath is made up to 200 25 liters.

After the usual subsequent treatment a brown is obtained.

Example 3.—400 gr. of 2-3-hydroxynaphthoic acid-m-nitranilide are dissolved with 30 800 gr. of Turkey-red oil in 1.5 liters of 38° Bé, caustic soda, diluted to a 200 liters bath and 4 liters of sulfite waste liquor are added.

35 10 kg. of cotton yarn or artificial silk yarn are introduced at 30° C. and 500 gr. of succinyl-diamino-anthrarufin and 600 gr. of concentrated hydrosulfite powder are added, and the material is dyed for a half hour after vatting, hung up, centrifuged and developed with the following solution:

40 250 gr. of 4-nitro-2-anisidine are introduced into 5 liters of cold water and 250 cc. of 20° Bé. hydrochloric acid are added. After solution, 90 gr. of sodium nitrite dissolved in about 500 cc. of cold water are 45 allowed to flow in and after 20 minutes it is neutralized with 180 gr. of sodium acetate dissolved in about 500 cc. of water and 180 gr. of aluminum sulfate dissolved in 1 liter of water, and then 6 kg. of Glauber's 50 salt are added. The bath is made up to 200 liters.

After the usual subsequent treatment a beautiful bluish-red is obtained.

Example 4.—600 gr. of diacetoacetyl-o-55 tolin are dissolved with 1 liter of Turkey-red oil in 1 liter of 40° Bé. caustic soda. Beforehand 3.75 kg. of 4,4'-dioxyindanthrene with 3.5 liters of 40° Bé. caustic soda, 2 kg. of concentrated hydrosulfite powder, 60 with the addition of 1 liter of Turkey-red oil, 8 liters of sulfite waste liquor and 800 gr. of soda are vatted and 25 kg. of piece goods are dyed at several ends at 40° C. for about 10 minutes. Then the above solution 65 is added and about 8 ends are further dyed.

Then the goods are well squeezed out and developed with the following 200 liter bath:

320 gr. of o-chloraniline are made into a paste with 2 liters of hot water and 360 cc. of 20° Bé. hydrochloric acid, dissolved 70 cold in 4.5 liters of water, cooled to 5° C. with ice and treated with 160 gr. of sodium nitrite dissolved in about 1.5 liters of water. After 15 minutes it is neutralized with 300 gr. of sodium acetate in 1.5 ltrs. of water 75 and 300 gr. of aluminum sulfate in 2.5 liters of water. Then 2.4 liters of 30° Bé. acetic acid, 6 kg. of Glauber's salt and 400 gr. of sodium bicarbonate are added.

After the usual subsequent treatment a 80 green is obtained.

Example 5.—De-gummed silk is ground- 85 ed for about 30 to 40 minutes at 25-30° C., with or without the addition of sodium chloride, with a solution which contains besides 2 gr. of 2-3-oxynaphthoic acid-p-anisidid and 1 gr. of the product known under the trade-mark "Protektol I, double powder" (compare color index 1924, page 363 and Fierz David, Technologie der Textilfasern 1926, volume 3, page 388, ac- 90 cording to which "Protectol" is obtainable by evaporating sulfite waste liquor) in ad- 95 dition 10% of the weight of silk per liter of dibenzoyl-4-8-diaminoanthrarufin paste, which has previously been vatted in a stand- 100 ard vat with 10 cc. of 30° Bé. caustic soda and 3 gr. of hydrosulfite. The goods are thor- 105oughly centrifuged, during which op- eration the vat-dyestuff is oxidized and de- 110 veloped with a diazo solution which con- 115 tains 2 gr. of p-nitro-o-anisidin and 20 cc. of 50% acetic acid per liter. Then it is rinsed, soaped at a boiling temperature with Marseilles soap, rinsed, brightened in the usual manner and dried.

A Bordeaux shade of extraordinary fast- 120 ness is obtained.

Example 6.—De-gummed silk or yarn is 110 grounded at 45° C. in a bath which contains in 1 liter 5 gr. of diacetoacetyl-o-tolidin, 3 cc. of Turkey-red oil, 35 cc. of 30° Bé. caustic soda, 2 gr. of "Protektol I, double powder," 10 gr. of indanthrene blue-green B paste, and 3 gr. of hydrosulfite. After three-quarters of an hour of good manip- 115 ulation it is well centrifuged and then de- 120 veloped with a diazo solution which contains in 1 liter the diazo compound from 2 gr. of o-chloraniline, 40 cc. of 50% acetic acid and 20 gr. of sodium chloride. After half an hour it is thoroughly rinsed, soaped at a boiling temperature and brightened as usual.

A brilliant green of extraordinary fast- 125 ness results.

I claim:

1. Process of dyeing cotton, artificial silk, and silk with vat and azo dyestuffs, which 130 comprises grounding the goods with an azo

component and at the same time with a vat dyestuff dissolved without esterification, and converting the vat dyestuff into the insoluble form by oxidation, and developing 5 the ice color on the fiber by means of a diazo solution.

2. Material dyed by the process of claim 1.

3. Process of dyeing cotton, artificial silk, and silk with vat and azo dyestuffs, which 10 comprises grounding the goods with a substantive arylid of an organic acid as azo-component and at the same time with a vat dyestuff dissolved without esterification, and converting the vat dyestuff into the insoluble form by oxidation, and developing 15 the ice color on the fiber by means of a diazo solution.

4. Material dyed by the process of claim 3.

5. Process of dyeing cotton, artificial silk, and silk with vat and azo dyestuffs, which 20 comprises grounding the goods with an acyl

acetic acid arylid and at the same time with a vat dyestuff dissolved without esterification, and converting the vat dyestuff into the insoluble form of oxidation, and developing 25 the ice color on the fiber by means of a diazo solution.

6. Material dyed by the process of claim 5.

7. Process of dyeing cotton, artificial silk, and silk with vat and azo dyestuffs in green 30 shades, which comprises grounding the goods with diacetoacetyl-o-tolidin and at the same time with a vat dyestuff of the indanthrene blue group dissolved without esterification and converting the vat dye- 35 stuff into insoluble form by oxidation, and developing the ice color on the fiber by means of a solution of a diazo chlorbenzol.

8. Material dyed by the process of claim 7.

In testimony whereof, I affix my signature. 40

WILHELM WINTERHALDER.